

H. S. REED AND H. L. PUBLOW,  
 PROCESS AND APPARATUS FOR THE PRODUCTION OF LEAD OXID,  
 APPLICATION FILED SEPT. 17, 1920.

1,376,581.

Patented May 3, 1921.



FIGURE 4



Witnesses

Fred Ulrich  
 M. Louise Thurston

By

Inventors  
 Harry S. Reed  
 Henry L. Publow  
 Chappell Pearl  
 Attorneys

# UNITED STATES PATENT OFFICE.

HARRY S. REED AND HENRY L. PUBLLOW, OF EAST LANSING, MICHIGAN.

## PROCESS AND APPARATUS FOR THE PRODUCTION OF LEAD OXID.

1,376,581.

Specification of Letters Patent.

Patented May 3, 1921.

Application filed September 17, 1920. Serial No. 411,013.

To all whom it may concern:

Be it known that we, HARRY S. REED and HENRY L. PUBLLOW, citizens of the United States, residing at East Lansing, county of Ingham, and State of Michigan, have invented certain new and useful Improvements in Processes and Apparatus for the Production of Lead Oxid, of which the following is a specification.

10 This invention relates to a process for the production of lead oxid from basic carbonates of lead containing organic matter or admixed with organic matter, and the apparatus for carrying out such process.

15 The invention is of particular consequence in the lead process for the recovery of sucrose from molasses. The great advantage is that it enables the complete recovery of lead in a superior form for use in said lead process.

20 The invention is of course of advantage or may be of advantage in other processes but is of particular advantage in the process indicated.

25 The object of the invention is to provide an efficient process and apparatus for the recovery or production of lead oxid from basic carbonates of lead, as indicated. Objects which pertain to details and economies of construction and operation will definitely appear from the detailed description to follow.

30 We accomplish the objects of our invention by the devices and means described in the following specification. The invention is clearly defined in the claims.

35 We carry out the improved process by the apparatus illustrated in the accompanying drawing, forming a part of this specification, in which:

Fig. I is a longitudinal detail sectional elevation view of the improved oxidizing furnace, taken on line 1—1 of Fig. II.

Fig. II is a detail transverse sectional elevation view through the oxidizing furnace, taken on line 2—2 of Fig. I.

40 Fig. III is a diagrammatic detail longitudinal sectional view through the disassociating furnace, taken on line 3—3 of Fig. IV.

Fig. IV is a transverse detail sectional view through the disassociating furnace, taken on line 4—4 of Fig. III.

In the drawings the sectional views are taken looking in the direction of the little arrows at the ends of the section lines and 55 similar numerals of reference refer to similar parts throughout the several views.

Considering the numbered parts of the drawing, 1 is the shell of the oxidizing furnace provided with a usual construction of vertically sliding doors 2 through the center of which is a usual construction of testing port 3. An air inlet passage 4 with a series of upwardly opening inlets 5, 5, 5 is in the bottom of the furnace. A vent 6 is provided in the upper part of the furnace. A revolving drum 7 is disposed longitudinally within the furnace on roller supports 8, 8, which are driven by the pulley 9.

The furnace is heated by electric heating units 10, 10 preferably disposed at each side of the drum. Pyrometers 11, 11 are provided in the upper part of the furnace chamber, and a pyrometer 12 is located centrally in the revolving drum.

The disassociating furnace comprises a shell 13 within which is disposed a hollow drum 14 carried on suitable rollers 15, 15 driven by any suitable means for revolving the same. The drum 14 is slightly inclined to advance the contents through the furnace as the drum is slowly rotated. Electric heating units 16 are disposed entirely around the central part of the drum 14 and partition plates 17 and 17 are at each end of the heating units to retain and conserve the heat.

A hopper 19 with spout 20 delivering into the drum 14 is at the intake end of this furnace, and a receiving bin 21 is at the opposite end to receive the treated material. An outlet 22 is provided for collecting the carbonic dioxid that is developed by the process, conserving the same for use particularly in the lead process above referred to. This furnace is provided with a pyrometer 23 centrally disposed within the hollow drum 14.

In carrying out our improved process we first dry the mass containing the basic carbonates of lead and organic material and then pulverize it so that the mass will pass through a ten mesh sieve. The same could be somewhat finer or coarser. However, fine particles are likely to be wasted by being blown away as dust and coarse particles are more difficult to handle in subsequent operations. A charge of the granular mass containing the dried basic carbonates of lead is then introduced into the mixing drum 7 of the oxidizing furnace. This is kept in a slow rotation to tumble the mass over. The furnace is maintained regularly at a temperature of about 600 degrees Fahr. The introduction of the cold tumbling barrel and

105

100

110

its contents drops the temperature which is gradually raised during the process to the temperature of the furnace. It has been found that this temperature should not exceed 750 degrees Fahr., for the reason that above that temperature the tendency is to the reduction to metallic lead by the organic matter. The range of temperature which secures the best result is from about 400 degrees to 600 degrees Fahr. The air containing the oxygen moves very slowly through the furnace, it not being necessary to provide a stack or any other means of forced draft.

The time consumed in the process for the treatment of this material in the lead process above referred to is about 45 minutes when using the apparatus shown. The material is tested by taking a spoonful and subjecting it to a temperature above that necessary for the disassociating of the basic carbonate of lead. This step of the process is considered complete if no metallic lead appears when thus tested.

When this step of the process is complete, as indicated above, the charge is withdrawn and the treated material is passed to the disassociating furnace illustrated in Figs. III and IV. The charge is introduced into the hopper 19 filling the same quite full so that it acts as a plug to prevent escape of the contained gases within the furnace. The material discharges through the spout 20 either by being poked by hand or by a suitable conveyer, not illustrated, into the revolving drum 14. It is here subjected to a temperature of from 1100 degrees to 1200 degrees Fahr. The temperature should not exceed a temperature slightly below the fusing point of lead oxid (PbO), that is, approximately 1600 degrees Fahr. This is to avoid fusing the contents of the furnace into an unwieldy mass.

The basic carbonates of lead by this treatment are decomposed into the lead oxid (PbO) and carbonic acid gas ( $CO_2$ ) and water ( $H_2O$ ). The carbonic acid gas is collected at the port 22. In the lead process above referred to it is passed to the carbonation tanks and used with or without any intermediate storing.

The interior of this furnace is filled with highly heated inert carbonic acid gas as soon as the operation is in full progress. This is of advantage in the disassociating step of the process. This protects the parts from undue corrosion as well.

The material, in passing through the drum 14, is thus completely disassociated. The lead oxid is discharged into the collecting bin 21.

Having thus described our invention, what we claim as new and desire to secure by Letters Patent is:

1. The process for producing lead oxid from basic carbonates of lead containing or

admixed with organic matter consisting in drying the mass, reducing the same to granular form, introducing the mass into a revolving drum in a vented electric furnace, agitating and heating the same in the presence of the contained air to a temperature of about 600 degrees Fahr. to slowly oxidize the organic matter, until a test portion heated above the disassociating temperature of the basic carbonate of lead shows no reduction to metallic lead, introducing the treated mass into a closed electric furnace having a discharge opening for the carbonic acid gas and having a revolving drum for advancing and agitating the contents, and a collecting bin for the lead oxid, and heating the same to a temperature of 1100 degrees to 1200 degrees Fahr. whereby the mass of material is heated within an atmosphere of carbon dioxide, whereby the material is disassociated into lead oxid (PbO), in granular form, carbonic acid gas and water, as specified.

2. The process for producing lead oxid from basic carbonates of lead containing or admixed with organic matter consisting in drying the mass, reducing the same to granular form, agitating and heating the same in a vented electric furnace in the presence of the contained air to a temperature of about 600 degrees Fahr. to slowly oxidize the organic matter, until a test portion heated above the disassociating temperature of the basic carbonate of lead shows no reduction to metallic lead, introducing the treated mass into a closed electric furnace having a discharge opening for the carbonic acid gas and having a revolving drum for advancing and agitating the contents, and a collecting bin for the lead oxid, and heating the same to a temperature of 1100 degrees to 1200 degrees Fahr. whereby the mass of material is heated within an atmosphere of carbon dioxide, whereby the material is disassociated into lead oxid (PbO), in granular form, carbonic acid gas and water, as specified.

3. The process for producing lead oxid from basic carbonates of lead containing or admixed with organic matter consisting in drying the mass, reducing the same to granular form, agitating and heating the same in a vented electric furnace in the presence of the contained air to a temperature of about 600 degrees Fahr. to slowly oxidize the organic matter, until a test portion heated above the disassociating temperature of the basic carbonate of lead shows no reduction to metallic lead, introducing the treated mass into a closed electric furnace having a discharge opening for the carbonic acid gas, and agitating and heating the same to a temperature of 1100 degrees to 1200 degrees Fahr. whereby the mass of material is heated within an atmosphere of carbon dioxide,

- whereby the material is disassociated into lead oxid (PbO), in granular form, carbonic acid gas and water, as specified.
4. The process for producing lead oxid from basic carbonates of lead containing or admixed with organic matter consisting in drying the mass, reducing the same to granular form, agitating and heating the same in a vented electric furnace in the presence of the contained air to a temperature of about 600 degrees Fahr. to slowly oxidize the organic matter, until a test portion heated above the disassociating temperature of the basic carbonate of lead shows no reduction to metallic lead, introducing the treated mass into a closed electric furnace having a discharge opening for the carbonic acid gas, and heating the same to a temperature of 1100 degrees to 1200 degrees Fahr. whereby the mass of material is heated within an atmosphere of carbon dioxid, whereby the material is disassociated into lead oxid (PbO), in granular form, carbonic acid gas and water, as specified.
5. The process for producing lead oxid from basic carbonates of lead containing or admixed with organic matter consisting in drying the mass, reducing the same to granular form, agitating and heating the same in a vented electric furnace in the presence of the contained air to a temperature of about 600 degrees Fahr. to slowly oxidize the organic matter, until a test portion heated above the disassociating temperature of the basic carbonate of lead shows no reduction to metallic lead, introducing the treated mass into a closed electric furnace having a discharge opening for the carbonic acid gas, and heating the same to a temperature of 1100 degrees to 1200 degrees Fahr. whereby the material is disassociated into lead oxid (PbO), in granular form, carbonic acid gas and water, as specified.
6. The process for producing lead oxid from basic carbonates of lead containing or admixed with organic matter consisting in drying the mass, reducing the same to granular form, agitating and heating the same in a vented electric furnace in the presence of the contained air to a temperature of about 600 degrees Fahr. to slowly oxidize the organic matter, until a test portion heated above the disassociating temperature of the basic carbonate of lead shows no reduction to metallic lead, introducing the treated mass into a closed electric furnace having a discharge opening for the carbonic acid gas, and heating the same to a temperature of 1100 degrees to 1200 degrees Fahr. whereby the material is disassociated into lead oxid (PbO), in granular form, carbonic acid gas and water, as specified.
7. The process for producing lead oxid from basic carbonates of lead containing or admixed with organic matter consisting in drying the mass, reducing the same to granular form, agitating and heating the same in a vented electric furnace in the presence of the contained air to a temperature of about 600 degrees Fahr. to slowly oxidize the organic matter, until a test portion heated above the disassociating temperature of the basic carbonate of lead shows no reduction to metallic lead, and heating the treated mass to a temperature of 1100 degrees to 1200 degrees Fahr., whereby the material is disassociated into lead oxid (PbO), in granular form, carbonic acid gas and water, as specified.
8. The process for producing lead oxid from basic carbonates of lead containing or admixed with organic matter consisting in drying the mass, reducing the same to granular form, agitating and heating the same in a vented electric furnace in the presence of the contained air to a temperature of about 600 degrees Fahr. to slowly oxidize the organic matter, until a test portion heated above the disassociating temperature of the basic carbonate of lead shows no reduction to metallic lead, and heating the treated mass to a temperature of 1100 degrees to 1200 degrees Fahr., whereby the material is disassociated into lead oxid (PbO), in granular form, carbonic acid gas and water, as specified.
9. The process for producing lead oxid (PbO) from basic carbonates of lead containing or admixed with organic matter consisting in reducing the same to granular form, agitating the same in a vented electric furnace and heating the same in the presence of the contained air to slowly oxidize the organic matter until the same is substantially eliminated, introducing the treated mass into a closed electric furnace having a discharge opening for the carbonic acid gas, and heating the same sufficiently to disassociate the mass into lead oxid (PbO), carbonic acid gas (CO<sub>2</sub>) and water (H<sub>2</sub>O), without raising the temperature sufficiently to fuse the said lead oxid.
10. The process for producing lead oxid (PbO) from basic carbonates of lead containing or admixed with organic matter consisting in reducing the same to granular form, agitating the same in a vented electric furnace and heating the same in the presence of the contained air to slowly oxidize the organic matter until the same is substantially eliminated, introducing the treated mass into a closed electric furnace having a discharge opening for the carbonic acid gas, and heating the same sufficiently to disassociate the mass into lead oxid (PbO), carbonic acid gas (CO<sub>2</sub>) and water (H<sub>2</sub>O).
11. The process for producing lead oxid (PbO) from basic carbonates of lead containing or

- 4
- taining or admixed with organic matter consisting in reducing the same to granular form, agitating the same in a vented electric furnace and heating the same in the presence of the contained air to slowly oxidize the organic matter until the same is substantially eliminated, then heating the same sufficiently to disassociate the mass into lead oxid (PbO), carbonic acid gas (CO<sub>2</sub>) and water (H<sub>2</sub>O).
12. The process for producing lead oxid (PbO) from basic carbonates of lead containing or admixed with organic matter consisting in reducing the same to granular form, agitating the same in a vented electric furnace and heating the same in the presence of the contained air to slowly oxidize the organic matter until the same is substantially eliminated, then heating the same sufficiently to disassociate the mass into lead oxid (PbO), carbonic acid gas (CO<sub>2</sub>) and water (H<sub>2</sub>O).
13. The process for producing lead oxid (PbO) from basic carbonates of lead con-

taining or admixed with organic matter consisting in heating the same in the presence of the contained air to slowly oxidize the organic matter until the same is substantially eliminated, then heating the same sufficiently to disassociate the mass into lead oxid (PbO), carbonic acid gas (CO<sub>2</sub>) and water (H<sub>2</sub>O).

14. An apparatus for treating basic carbonates of lead containing or admixed with organic matter, comprising a vented electric furnace, with a revolving drum therein, a closed electric furnace having a port for collecting the carbon dioxide gas, with an inclined revolving drum therein, with a hopper delivering into one end of said drum, and a bin for collecting the lead oxid.

In witness whereof, we have hereunto set our hands and seals in the presence of two witnesses.

HARRY S. REED. [L. S.]  
HENRY L. PUBLLOW. [L. S.]

Witnesses:

LUELLA G. GREENFIELD,  
MARGARET L. GLASGOW.